

## UNITED STATES PATENT OFFICE

TAGE F. WERME, OF FAIRFIELD, CONNECTICUT, ASSIGNOR TO REMINGTON ARMS COMPANY, INC., A CORPORATION OF DELAWARE

## AMMUNITION

No Drawing. Application filed November 19, 1927. Serial No. 234,553.

This invention relates to ammunition, particularly small arms ammunition, and has for its object the provision of ammunition such that erosion and corrosion of the bore of the gun barrel will be eliminated or reduced to a minimum. It is well known among the users of firearms that ordinary ammunition is very destructive of the surface of the bore of the gun in which it is fired, corrosion and pitting of the bore taking place within a few hours unless the gun is carefully cleaned. Even thorough cleaning by the usual methods is ineffective to prevent corrosion. At the present time, corrosion is especially destructive of guns which shoot "center fire" ammunition, a noncorrosive "rim fire" ammunition being now available. By the present invention, noncorrosive center fire as well as rim fire ammunition becomes possible.

20 It has long been thought and is now universally recognized as true, that corrosion is due to residues left in the bore by the combustion of the propellant powder, and the priming mixture used to ignite the powder.

25 Potassium chlorate contained in either the powder or the priming mixture is the agent which is chiefly, if not entirely, responsible for corrosion. On the firing of the charge, the potassium chlorate yields oxygen leaving 30 a residue of highly hygroscopic potassium chloride, which is driven by the high pressures prevailing in the gun barrel into microscopic fissures and indentations in the bore, from which it cannot be removed by 35 mechanical swabbing or by the use of the ordinary so-called gun cleaning compositions, since it is insoluble in the fluids contained in such compositions. The present invention 40 contemplates protecting the bore of the gun from corrosion by coating the bore with a substance which will fill and close any tool marks or indentations in the bore as well as coating the entire surface of the bore with a film which is both impervious to moisture and 45 prevents the contact of destructive chloride or other residues with the surface of the steel.

Lead or its compounds are utilized for this purpose. A prior patent discloses the use of lead oxide for this purpose. The invention 50 of said patent, however, contemplated the ad-

dition of a lead salt, preferably lead nitrate, to the priming mixture, and the use of such a priming composition with ordinary propellant powder. The use of a lead salt in the priming composition, however, has certain disadvantages. For example, substantially all priming compositions now in use contain mercury fulminate and in the intimate mixtures of the ingredients necessary for proper priming, compositions containing 55 both lead nitrate and mercury fulminate were found to deteriorate with time and exposure to a moist atmosphere. The addition of stabilizing ingredients to prevent such deterioration presents substantial difficulties, 60 since the volume of priming mixture which can be placed in small arms ammunition, especially small arms ammunition manufactured in accordance with the quantity 65 production methods universally used in this country, is very limited. The present invention therefore contemplates the addition 70 of lead dust or certain lead compounds to the propellant powder.

It has been discovered that when lead dust 75 in quantities up to 12% by weight is added to the propellant powder a coating is formed on the bore of the gun which substantially eliminates corrosion. It is thought that this coating may be, in part at least, an amalgam 80 of mercury and lead, the mercury being supplied by the decomposition of the mercury fulminate contained in the priming mixture. The coating thus formed adheres well to the 85 surface of the steel, and forms an excellent protection against corrosion. Barrels in which my improved ammunition has been fired have withstood very severe moisture tests with no sign of rust or pitting. Moreover, the coating material does not accumulate 90 in the bore, or interfere with its accuracy after long continued firing. Any excess of the coating material appears to be removed by the passage of the bullet or blown out with the powder blast, and the accuracy 95 is never impaired.

The lead dust may be incorporated with the powder in the course of its manufacture or may be subsequently added to the powder at any stage in the loading of the cartridge. 100

Compounds of lead such for example as lead oxide, may be used in place of metallic lead with excellent results.

Applicant being the first to discover that corrosion may be reduced or eliminated by the admixture of lead or its compounds with the propellant powder of small arms ammunition, the appended claims are to be broadly construed.

10 What is claimed is:

1. The method of producing a cartridge capable of preventing corrosion in the bore of the gun in which the cartridge is to be fired, which comprises intermixing with the propellant charge a quantity of lead dust capable of forming a corrosion preventing coating in the bore of the gun when the cartridge is fired therein.
2. The method of preventing corrosion in the bore of a gun, comprising the incorporation in the propellant powder of a cartridge of a quantity of lead dust, and then forming a corrosion preventing coating containing such lead in the bore by firing the said cartridge in the gun.
3. A small-arms cartridge containing a propellant powder in which lead dust is intermixed in a quantity sufficient to form a corrosion preventing coating in the bore of the gun in which the cartridge is fired.
4. A small-arms cartridge containing a propellant charge in which lead dust is intermixed in a quantity up to 12% by weight of the charge to form a corrosion preventive coating in the bore of the gun in which the cartridge is fired.

TAGE F. WERME.

.0

5

0

5

0

5